

United States Patent [19]  
Winslow

[11] 3,847,612  
[45] Nov. 12, 1974

[54] **LIGHT-SENSITIVE HEAT-DEVELOPABLE SHEET MATERIAL**

[75] Inventor: **John M. Winslow**, St. Paul, Minn.

[73] Assignee: **Minnesota Mining and Manufacturing Company**, St. Paul, Minn.

[22] Filed: **Feb. 2, 1973**

[21] Appl. No.: **329,107**

[52] U.S. Cl. .... **96/67**, 96/114.1, 96/114.6

[51] Int. Cl. .... **G03c 1/02**

[58] Field of Search .... 96/67, 52, 58, 114.1, 114.6; 117/36.7-36.9

[56] **References Cited**

UNITED STATES PATENTS

3,080,254 3/1963 Grant, Jr. .... 117/36.8

3,218,166 11/1965 Ritter ..... 96/67  
3,589,903 6/1971 Birkeland ..... 96/67

Primary Examiner—David Klein  
Assistant Examiner—Alfonso T. Suro Pico  
Attorney, Agent, or Firm—Alexander, Sell, Steldt & DeLaHunt

[57]

**ABSTRACT**

Dust formation is avoided and dense black images are obtained during heat development of exposed dry silver sheet materials by employing a synergistic combination of individually ineffective toner materials.

**6 Claims, No Drawings**

# LIGHT-SENSITIVE HEAT-DEVELOPABLE SHEET MATERIAL

This invention relates to photosensitive heat-developable dry silver sheet materials and has particular reference to improved means for obtaining images of desirable density and color.

Photosensitive heat-developable dry silver sheet materials, as described for example in U.S. Pat. No. 3,457,075, contain a photosensitive silver halide catalyst-forming means in catalytic proximity with a heat-sensitive combination of organic silver salt and reducing agent. Particularly where the reducing agent is a hindered phenol, it is found desirable to include an image intensifier or toner material, of which phthalazinone has been an outstanding example.

Phthalazinone and various other materials have previously been employed as toners in light-stable heat-sensitive copy-sheets based on organic silver salts and reducing agents. Phthalazinone is a preferred material in compositions shown in U.S. Pat. No. 3,080,254; other materials therein disclosed, such for example as imidazole, must be employed in much larger amounts and are generally less effective. Both phthalic acid and phthalazinone are shown in U.S. Pat. No. 3,218,166 to be effective toners for heat-sensitive compositions containing organic silver salts and hindered phenolic reducing agents. However in dry silver sheet materials employing the hindered phenolic reducing agents and containing also a catalytic quantity of photosensitive silver halide, neither phthalic acid nor imidazole has been found effective in causing useful darkening of the image. Phthalazinone is fully effective in dry silver sheets both as an image toner and for other purposes, as noted for example in U.S. Pat. No. 3,589,903; but this compound has been found to cause slight dusting, which becomes noticeable during heat development of large numbers of the exposed sheets. The dust factor apparently is a result of sublimation of the toner material, the vapor then condensing on cooler portions of the developing apparatus. It has also been observed that dry silver sheets containing phthalazinone have a tendency to lose photosensitivity and to provide less desirable images when first subjected to prolonged storage at elevated temperature and humidity.

It has now been found possible to provide photosensitive heat-developable dry silver imaging sheets which give dense black images, retain full effectiveness during prolonged storage, and do not emit dust-forming vapors during development, by incorporating with the combination of silver halide, organic silver salt and hindered phenolic reducing agent significant small amounts of each phthalic acid and imidazole.

As previously indicated, neither of these materials is at all effective by itself as an image toner for these dry silver sheet materials; yet the two together are found to be fully as effective as phthalazinone in providing image areas of desirable cold tone and this ability is maintained during prolonged storage.

Phthalic acid may effectively be replaced in whole or in part by corresponding molar amounts of naphthalene-2,3-dicarboxylic acid or of o-phthalamic acid. Each of these compounds will be seen to be capable of condensation to form a five-membered heterocyclic ring structure.

Somewhat analogously, substituted imidazoles having the 5-membered heterocyclic imidazole ring struc-

ture are also found to be useful. Exemplary of such compounds are benzimidazole, 5,6-dimethylbenzimidazole, 2-methylbenzimidazole, 2-hydroxybenzimidazole.

The amount of toner materials required will vary with the proportion of silver salts and other reactants as well as with the thickness of the coating. Good results have been obtained in a specific example using about 22 parts by weight of phthalic acid and about 15 parts by 10 weight of imidazole in a coating prepared with about 225 parts of silver behenate half soap, 155 parts of hindered phenolic reducing agent, and 480 parts of resinous binders, applied at a dry coating weight, after removal of volatile liquid vehicle, of about ten grams per 15 square meter. In another example, 50 parts by weight of phthalic acid and 10 parts of benzimidazole are found to be effective in a transparent coating prepared with approximately 715 parts of silver behenate full soap, 1,000 parts of resinous binders, and 770 parts of 20 hindered phenolic reducing agent, applied at 19 grams per sq. meter.

The coating made with the half soap, containing 14.5 percent silver, may be shown by calculation to contain 25 0.44 mole of phthalic acid and 0.73 mole of imidazole per mole of silver. Similarly, the transparent coating containing the full soap may be shown to contain 0.18 mole of phthalic acid and 0.057 mole of benzimidazole 30 per mole of silver. More broadly, it has been found possible to obtain distinct improvement in image appearance with dry silver coatings based on organic silver salts and hindered phenolic reducing agents by incorporating as toner materials an imidazole and phthalic acid or equivalent in amounts within the approximate range of 0.04 to 0.8 mole of the acid and 0.02 to 1.4 35 moles of the imidazole per mole of total silver. A preferred range is about 0.15 to 0.5 mole of acid and 0.1 to 0.7 mole of imidazole per mole of silver. In these 40 coatings it will be recognized that some minor amount, not more than about ten percent, of the total silver will be present as photosensitive silver halide, the remainder being light-stable organic silver salt.

Some improvement in image appearance may be 45 achieved in accordance with the principles of the invention when using other hindered phenolic reducing agents, such for example as those listed in the aforementioned U.S. Pat. No. 3,218,166; but the best image appearance has been realized when using as the reducing agent the compound 2,6-methylene-bis(2-hydroxy- 50 3-tertiarybutyl-5-methylphenyl)-4-methylphenol, a commercial form of which is also known as "Plastanox 80" antioxidant; and this substance is presently greatly preferred in the sheet materials of this invention.

For use on paper or other non-transparent backings 55 it is found convenient to use silver half-soaps, of which an equimolar blend of silver behenate and behenic acid, prepared by precipitation from aqueous solution of the sodium salt of commercial behenic acid and analyzing about 14.5 percent silver, represents a preferred 60 example. Transparent sheet materials made on transparent film backings require a transparent coating and for this purpose the silver behenate full soap, containing not more than about four or five percent of free behenic acid and analyzing about 25.2 percent silver, may be used. Other components, such for example as colorings, opacifiers, extenders, spectral sensitizing dyes etc. 65 may be incorporated as required for various specific purposes.

The following examples are offered for further illustration, but not as limitation, of the principles of the invention. Proportions are in parts by weight unless otherwise noted.

## EXAMPLE 1

Silver behenate half soap is homogenized in acetone and then diluted with further acetone and toluene to the formula

|           |             |
|-----------|-------------|
| half soap | 10.83 parts |
| acetone   | 58.94       |
| toluene   | 30.23       |

To 80.85 grams of the homogenate is added, under 15 darkroom conditions,

|                                                 |            |
|-------------------------------------------------|------------|
| acetone                                         | 6.37 grams |
| polyvinyl butyral ("B-76" resin)                | 10.40 gm.  |
| 3% solution of mercuric acetate in methanol     | 1 ml.      |
| 5% solution of calcium bromide in methanol      | 1 ml.      |
| hindered phenolic reducing agent (Plastanox 80) | 6 grams    |

and the mixture is coated on paper pre-treated with polyvinyl alcohol. The coating weight after drying is seven grams per square meter.

A second composition is prepared by first mixing together

|                   |             |
|-------------------|-------------|
| acetone           | 339.9 grams |
| methanol          | 118.5       |
| cellulose acetate | 25.0        |
| colloidal silica  | 3.5         |

To 100 grams of the mixture is then added

|                                       |         |
|---------------------------------------|---------|
| 0.25% Victoria Blue dye in methanol   | 0.1 ml. |
| 0.05% spectral sensitizer in methanol | 1.5 ml. |
| phthalic acid                         | 0.6 gm. |
| imidazole                             | 0.4 gm. |

The mixture is applied over the previous layer and dried. The dry coating weight is 2.7 grams/sq.m. The spectral sensitizer is 1-methyl-3-allyl-5[ (3-ethyl-2-benzoxazolinylidene) ethylidene]-2-thiohydantoin. The molar ratios of phthalic acid and imidazole to total silver are 0.37 and 0.71 respectively.

A sample is exposed sensitometrically and is developed by heating for three seconds at 260°F. with results as follows:

| $D_{min}$ | $D_{max}$ | gamma | speed | image |
|-----------|-----------|-------|-------|-------|
| .19       | 1.28      | 1.35  | 1.0   | black |

Speed is here defined as  $1000/E_{0.6}$  where  $E_{0.6}$  represents meter candle seconds of exposure required to achieve a density of 0.6 above base plus fog.

A large quantity of coated paper prepared as just described is exposed and developed in a commercial copying machine operating under the conditions indicated, with complete freedom from dusting.

Another sample of the sheet material of Example 1 is first subjected to accelerated aging conditions of 80°F. and 80% relative humidity for a period of three months, and is then exposed, developed and tested as before, with results as follows:

| $D_{min}$ | $D_{max}$ | gamma | speed | image color |
|-----------|-----------|-------|-------|-------------|
| .13       | 1.30      | 1.20  | 1.20  | black       |

The test conditions, which are sufficiently severe to cause significant deterioration of properties in sheets prepared with phthalazinone, are seen to have very little if any adverse effect on the product of the present example.

## EXAMPLE 2

A homogenate is prepared of

|                           |         |
|---------------------------|---------|
| silver behenate full soap | 100 gm. |
| methyl isobutyl ketone    | 54      |
| toluene                   | 175     |
| methyl ethyl ketone       | 501     |

20 To 72 grams of the homogenate is added acetone

|                                              |          |
|----------------------------------------------|----------|
| acetone                                      | 14.4 gm. |
| mercuric bromide (as .5% soln. in methanol)  | .0045    |
| mercuric acetate (as 2.5% soln. in methanol) | .216     |
| polyvinyl butyral                            | 9.2      |
| vinyl resin ("VAGH")                         | 1.8      |
| Sudan yellow (as .05% soln. in methanol)     | .015     |

The vinyl resin is a copolymer, of vinyl acetate and 30 vinyl chloride, containing hydroxyl radicals.

The Sudan yellow dye is optional

The mixture is prepared under darkroom conditions. It is coated on transparent polyester film to a coating weight, after drying, of 16.2 gm/sq.m.

35 A second composition is prepared using

|                                                |        |
|------------------------------------------------|--------|
| toluene                                        | 34 gm. |
| methyl ethyl ketone                            | 32     |
| methanol                                       | 22     |
| vinyl chloride-vinyl acetate copolymer ("VYH") | 6      |
| tetrachlorophthalic anhydride                  | .43    |
| phthalic acid                                  | 2.2    |
| benzimidazole                                  | .43    |
| phenolic reducing agent of Example 1           | 3.42   |
| antistatic agent (optional) ("Catanac SN")     | .43    |

45 and is applied over the first coat at a coating weight, after drying, of 2.7 grams/sq.m. The molar ratios of phthalic acid and benzimidazole to total silver are 0.167 and 0.046 respectively.

The film is exposed through a 0-4 continuous wedge 50 to illumination from a carbon arc and developed by holding for 30 seconds in a bath of inert fluorocarbon liquid maintained at 260°F. The sensitometric values attained are:

| $D_{min}$ | $D_{max}$ | gamma | image color |
|-----------|-----------|-------|-------------|
| .08       | 2.60      | 2.0   | blue-black  |

55 What is claimed is as follows:

1. A photosensitive heat-developable sheet material having an image-forming stratum comprising (1) photo-sensitive silver halide catalyst-forming means and (2) heat-sensitive reactant image-forming means including an organic silver salt oxidizing agent and a hindered phenolic reducing agent for silver ion, the oxidation-reduction reaction of which to produce a visible change is accelerated by said catalyst, and (3) as

image intensifier material, a mixture of (a) one or more of the compounds phthalic acid, naphthalene-2,3-dicarboxylic acid, or phthalamic acid, and (b) an imidazole.

2. Sheet material of claim 1 wherein said hindered phenolic reducing agent is 2,6-methylene-bis(2-hydroxy-3-tertiary-butyl-5-methylphenyl)-4-methylphenol.

3. Sheet material of claim 1 wherein said intensifier material is constituted of 0.04 to 0.8 mole of said acid and 0.02 to 1.4 moles of said imidazole per mole of total silver.

4. Sheet material of claim 3 wherein said image inten-

sifier material consists of phthalic acid and imidazole.

5. Sheet material of claim 3 wherein said image intensifier material consists of phthalic acid and benzimidazole.

6. Sheet material of claim 1 wherein said hindered phenolic reducing agent is 2,6-methylene-bis(2-hydroxy-3-tertiarybutyl-5-methylphenyl)-4-methylphenol and said image intensifier material consists of 0.15 to 0.5 mole of phthalic acid and 0.04 to 0.7 mole of imidazole or benzimidazole per mole of total silver.

\* \* \* \* \*

15

20

25

30

35

40

45

50

55

60

65